

Patented Oct. 8, 1946

2,409,094

## UNITED STATES PATENT OFFICE

2,409,094

## BALLAST BLOCK

Carl C. Ahles, Albany, N. Y.

No Drawing. Application May 29, 1943,  
Serial No. 489,257

4 Claims. (Cl. 106—97)

1

My invention relates to ballast blocks, counterweights and the like, and particularly to articles of this type which are magnetic to facilitate the handling thereof by electromagnets, and which are cold molded or cast, like concrete, to form a strong, dense mass of exceptionally high specific gravity.

At the present time due to the great demand for iron and steel and other heavy metals in the production of war materials, substitutes for iron pigs and the like which have been heretofore used for ship ballast, counterweights, etc., have been sought. What is needed is a material of high specific gravity which can be utilized en masse, or in the form of blocks which can be conveniently handled and closely packed and which are formed of materials not so essential in the war effort as the various heavy metals. Ordinary concrete can of course be cast en masse or in the form of blocks and for these reasons would be an ideal material were it not for its comparatively low specific gravity and the difficulty of handling and placing preformed blocks made therefrom. Copper, lead, or other heavy slags might be used in the concrete as an aggregate instead of stone, but in crushing the same, insufficient fines are produced to use with the larger particles in order to make a dense concrete and hence, either a fine aggregate of substantially lower specific gravity, such as sand, must be used, or the expense of special fine crushing must be undertaken to produce a desirably dense concrete. Furthermore concrete blocks of such aggregate cannot be conveniently handled and are a poor substitute for iron pigs.

The principal objects of my invention are to provide a dense concrete structure having a very high specific gravity which is formed of materials available in many localities and which, moreover, will impart magnetic properties to the blocks made therefrom which will facilitate the handling and the packing of the same.

With these objects in view I have formed highly satisfactory ballast blocks from a concrete comprising, by weight, one part of hydraulic cement and from four to eight parts of magnetite. Such blocks are highly magnetic and thus may be easily handled by electromagnets. Magnetite is the magnetic oxide of iron ( $Fe_3O_4$ ) and, when pure, contains more than 72% of metal. The specific gravity is about 5.1. As found in nature, the magnetite may be combined with lighter, non-magnetic materials and the specific gravity may vary from about 4.2 to 5.1. However, as distinguished from slags, the magnetite, when crushed, pro-

duces a considerable quantity of fines which may be readily separated from the lighter materials by magnetic separators. Such fines are preferably used alone with the hydraulic cement to form concrete consisting entirely of fine aggregate and a binder, or, as a fine aggregate mixed with a coarse aggregate of magnetite. However, a satisfactory, heavy, magnetic concrete may be formed by combining a coarse, or a partly coarse and partly fine, heavy aggregate such, for example as heavy slag or ore, which may or may not be magnetic with a comparatively small proportion of fine magnetite. Of course the magnetic properties of the concrete will vary with the proportion of magnetic material therein but concrete in which magnetite constitutes 10% or more, by weight, of the total aggregate can be handled with the present types of magnetic equipment.

Because most of the lighter materials can be eliminated from the finely crushed ore and the resulting concrete is therefore of higher specific gravity, I prefer to use, as an aggregate, magnetite, 60% of which will pass a No. 10 sieve. The proportion of dry voids in such a mass is comparatively small, usually from 30 to 40%, and the cement which is required to fill these voids, and which is of course much lighter than the magnetite, does not reduce the specific gravity of the finished concrete to the same degree as would be the case with an aggregate having a greater proportion of voids. Only sufficient water to form a workable mix should be used.

Where the material is cast in the form of blocks which must be handled or shipped, as distinguished from casting en masse, I prefer to use from four to six parts by weight of magnetite to one part by weight of hydraulic cement because, when the magnetite ratio is appreciably increased the blocks are not so strong. If the blocks are subjected to a steam curing treatment they will, in twenty-four hours, develop a crushing strength of around three thousand pounds per square inch. Thus the blocks may be made one day and shipped the next. In twenty-eight days they will acquire a crushing strength of about four thousand pounds per square inch. In casting, the use of vibrating molds or other means for producing a dense structure are preferably employed.

While, as pointed out above, I prefer to form the blocks entirely of fine aggregate and hydraulic cement, because by finely crushing the ore a purer and heavier concentrate is obtained, it is to be understood that both the fine aggregate and the coarse aggregate may be magnetite. On the other hand, as pointed out above, aggregates of other

magnetite

heavy materials such, for example, as copper or lead slags may be used with a fine aggregate consisting in whole or in part of magnetite, and blocks made therefrom will be sufficiently magnetic to permit of their being handled by electromagnets. In any case however it should be borne in mind that a dense concrete of the heaviest materials is desired and the coarse and fine aggregate should be proportioned with this end in view so that the voids, which are necessarily filled with the cement which is very much lighter, are reduced to a minimum.

Ballast blocks made of finely crushed magnetite and Portland cement should weigh in excess of one hundred ninety pounds per cubic foot or, in other words, have a specific gravity of the order of about 3 or more; and, due to their regular size, they may be piled or packed very closely so that, when any given space is filled thereby, the aggregate weight is almost equal to that of the iron pigs which can be placed in said space.

By the term, "ballast block," as used in the claims, I mean to include both precast blocks of regular shape and concrete cast en masse.

What I claim is:

- 5 1. A magnetic ballast block having a specific gravity of the order of 3 and up and formed of concrete comprising, by weight, about one part of hydraulic cement and from about four to about eight parts of magnetite.
- 10 2. A magnetic ballast block having a specific gravity of the order of 3 and up and formed of concrete comprising, by weight, about one part of hydraulic cement and from about six to about eight parts of magnetite.
- 15 3. The structure set forth in claim 1 in which the cement is Portland cement.
- 20 4. The structure set forth in claim 2 in which the cement is Portland cement.

CARL C. AHLES.